

April 11, 1950

H. G. LYKKEN

2,503,555

## ORE CONDITIONING AND REDUCTION PROCESS

Filed Sept. 25, 1943

3 Sheets-Sheet 1



INVENTOR  
HENRY G. LYKKEN

By Paul, Paul & Moore  
ATTORNEYS

April 11, 1950

H. G. LYKKEN

2,503,555

## ORE CONDITIONING AND REDUCTION PROCESS

Filed Sept. 25, 1943

3 Sheets-Sheet 2



Fig. 2



Fig. 5

INVENTOR  
HENRY G. LYKKEN

By Paul, Paul & Moore  
ATTORNEYS

April 11, 1950

H. G. LYKKEN

2,503,555

ORE CONDITIONING AND REDUCTION PROCESS

Filed Sept. 25, 1943

3 Sheets-Sheet 3



## UNITED STATES PATENT OFFICE

2,503,555

ORE CONDITIONING AND REDUCTION  
PROCESS

Henry G. Lykken, Minneapolis, Minn.

Application September 25, 1943, Serial No. 503,795

12 Claims. (Cl. 75—39)

**1**

This invention relates to a process and apparatus for the heat treatment and processing of finely divided or pulverized ores such as carbonates, sulphides and sulphates to the oxides, but more particularly the invention relates to methods and apparatus for the partial deoxidation or partial reduction of finely divided iron ore for the purpose of concentration and, in a variation of the methods and apparatus, the invention provides for the complete reduction and smelting of such ores. The invention relates particularly to the metallization of iron ores having a percentage iron content below that which can be shipped economically to and utilized in blast furnaces. The invention provides for the reduction of such ores directly to the metallic state. It is an object of the invention to provide such methods and apparatus.

More particularly it is an object of the invention to provide improved apparatus and processes for treating finely divided ores, particularly low grade ores and more specifically to provide apparatus and processes for smelting or reducing such finely divided ores. It is a further object of the invention to provide apparatus and processes wherein finely divided ore is conditioned for concentration or smelting by utilizing radiant heat under reverberatory conditions. Other and further objects of the invention are those inherent in the apparatus and processes herein illustrated, described and claimed.

The invention is illustrated with reference to the drawings in which

Figure 1 is an elevational view representing a cross section through one form of furnace of the present invention utilized in carrying out the processes of the invention;

Figure 2 is a composite cross-sectional view of the furnace apparatus shown in Figure 1 at five different levels. Thus, the angular segment between the lines A—X and E—X is taken along the level A—A, the segment between the lines A—X and B—X is taken at the level B—B, the segment between the lines B—X and C—X is taken at the level C—C, the segment between the lines C—X and D—X is taken at the level D—D and the segment between the lines D—X and E—X is taken at the level E—E, all with reference to Figure 1;

Figure 3 is an enlarged fragmentary elevational view of the ore-feeding mechanism shown in Figure 2;

Figure 4 is an elevational, cross-sectional view through another form of apparatus of the invention utilized for smelting ore; and

**2**

Figure 5 is a composite, cross-sectional view wherein the segment shown around the arc F—G—H is taken at the level G—G of Figure 4 and the section around the arc H—K—F is taken at the level K—K of Figure 4. The sectional view of the lower portion of Figure 4 is along the lines 4—4 of Figure 5.

## ORE TREATING FURNACE

10 Referring to Figures 1, 2 and 3 the furnace illustrated is for the purpose of treating finely divided ores without causing any agglomeration of the finely divided particles, and for example may be used for converting finely divided hematite ores to the magnetite condition, prior to electromagnetic concentration, for the metallizing of iron ores, reduction of iron ore, partially or completely, to metallic iron, or may be used for the treatment of carbonate, sulphide or sulphate ores to oxidize them.

15 The apparatus of Figure 1 consists of a base generally designated 10 on which there is mounted a plurality of upright columns 11—11 which serve as the basic framework of the furnace. The framework serves to support a hopper generally designated 19, and ore-feeding mechanism 25, reverberatory furnace section 40, heat exchanger section 44 and ore-withdrawal apparatus 72.

20 At the top of the columns 11, there is a roof 12 which is provided with a spout 13 for the introduction of the incoming ore stream into the top of a hopper 19 which is formed by the wall plates 14 and the hopper bottom plates 15, 16, 17 and 18. The hopper inner plates 16 and 17 constitute a cone and with the downwardly converging conically shaped outer plates 15 and 16 serve to cause the ore generally designated O to be directed to a plurality of spouts 20 arranged in a circle at the bottom of the hopper. Any number of spouts 20 may be used around the circular bottom of the hopper and they deliver the ore into the hopper portion 22 of the ore-feeding mechanism generally designated 25.

25 The ore-feeding mechanism may be of any desirable type capable of feeding a thin "curtain" of ore particles downwardly into the furnace. The illustrated form of apparatus for accomplishing this process consists of a plurality of vane-type feeders illustrated between the lines A—X and E—X of Figure 2 and in detail in Figure 3. Thus, as illustrated in Figure 3, the hopper 22 of the ore-feeding mechanism generally designated 25 is provided with a plurality of semi-cylindrical bottoms 26 which extend radially with respect to the circular hopper 22. In

each of the circular bottoms 26 there is a thin narrow slit 24 in chute 30 which may be from one-half to one inch in width and of a length equal to the width of the hopper 22 in a radial direction. Each of the shafts 27 is provided with a gear 32 and the adjacent gears 32 are geared together by idlers 33. A motor generally designated 35 is shown in Figure 2 and is provided with a built-in or external gear box, and is attached to one of the shafts 27 for slowly rotating the shaft. The gear 32 on the motor-driven shaft serves to drive the adjacent gears 32 through the connected idler 33, and adjacent gears 32 in turn serve to drive still the next adjacent gears 32 through their connecting idlers, and so on for all of the shafts 27 in the group. This may be continued all around the entire circumference of the furnace ore feeder, but it is preferred to install the motor drives in "segments" so that the failure or clogging of one segment will not entirely interrupt the furnace. The ore feeders may be arranged circumferentially end to end so as to form a continuous or nearly continuous circle rather than a circle of radial slits, or they may be arranged along successive chords of the circle, one feeder overlapping the next to form a circle around the axis of the furnace.

The action of the ore feeder is as follows: The finely granulated ore drops into the space between the vanes 28 on shafts 27 and is then carried around by the vanes as the shafts are rotated. As the ore then reaches the thin slit 24 in the chute 30, the ore is brushed through the slit of each spout 30 until all of the ore between those particular vanes has been dropped, and then the ore between the next pair of vanes is similarly brushed through the slit 24 and drops into the furnace. This goes on continuously and as a result a "curtain" of ore particles falls continuously down through the furnace under the circle of spouts 30. The ore-feeding mechanism 25 is supported on the framework 23 as is also the upper portion of the reverberatory furnace section, generally designated 40.

The reverberatory furnace section 40 consists of a vertical cylinder 41 which may be of any suitable horizontal and vertical dimensions supported on the trusswork 23 and upon suitable brackets 42. In Figure 1, the break in the furnace section 40 is intended to designate variations in height to accommodate the heating requirements of different sizes of ores. The height of the reverberatory radiant heat furnace section 40 depends upon the size of the ore being treated, the flame temperature of operation and the reaction temperature to which the furnace feed particles (ore and carbonaceous material) are heated. A sufficient height of portion 40 is provided so as to allow the particles of ore and other material constituting the furnace feed to be heated to the required reaction temperature by radiant reverberatory energy while the particles are falling downwardly around the heat source 75. Where the particles are larger, or where a higher reaction temperature of the particles is sought, the furnace height is increased. Similarly, for finer particles or lower temperatures, the height may be decreased. The furnace is thus designed for ore of a particular size.

The heat source, illustrated as flame 75, radiates heat energy in all directions, and this is reflected by the walls of the furnace repeatedly, thus setting up a condition of reverberating heat energy within section 40. As each particle of

furnace charge falls downwardly, the reverberating energy is impinged against it, and heating of the particle thus results. As the particles are small and the amount of reverberating energy is large, heating is almost instantaneous. Energy waves that do not impinge upon the particles are not wasted, because they simply reflect from the refractory walls 46, top 48 and cone 52.

A shoulder is provided in the furnace at 43 where the diameter is reduced and from the shoulder 43 there extends another cylindrical section 45 which forms the outer wall of the heat absorber section 44. If desired, the outer dimensions of the cylinders 45 and 41 may be identical, although the shoulder 43 provides a convenient ledge for supporting the refractory brick-work of the furnace.

Within the section 41 there is provided a refractory brick-work 46 and the brick-work is extended across the top of the furnace as shown at 48. Suitable radial openings are provided in the brick-work to receive the bottom ends of each of the spouts 30—30 and a central opening is provided at 49 for receiving the heat source burner nozzle generally designated 50 and steam nozzle (not illustrated) where used. The space within the reverberatory furnace section 40 is the reacting zone in which the ore particles are heated and treated.

Below the furnace zone the refractory lining is formed into a converging cone 52 which terminates at the circular bottom opening 53. Support for the refractory lining 52 is provided by a plurality of boiler tubes constituting tube bank 54 of the heat absorber, generally designated 44. The tubes 54 extend from a circular steam drum 55 radially inwardly at 57, and thence downwardly and inwardly at 58. The tubes then continue downwardly at 59 until they reach the point 60 at which they diverge outwardly at 61 to the water drum 62. A sufficient number of boiler tubes 54 are provided so that at the vertical portion 59 they are spaced uniformly several inches apart as shown in the section between the lines C—X and D—X of Figure 2.

The lower portion of each boiler tube in bank 54 is provided with a fin 64 which extends from the boiler tube in the direction of the adjacent boiler tube as shown in the cross section between the lines D—X and E—X of Figure 2. The fins 64 are of sufficient width so that they close off the space between adjacent boiler tubes, and thus the tubes and the fins 64 form a continuous wall (see Figure 2) at the level E—E of Figure 1.

Under certain conditions of operation the gases passing out between tubes at 59, contain combustible constituents and have a sufficiently high temperature to ignite in the presence of oxygen. By increasing the distance between the inner bank of tubes 54 and the next bank of tubes 55, space is allowed for combustion of such constituents, which may be accomplished by introducing air into such enlarged space by suitable nozzles, not illustrated. In this way the entire heat value of the gases is recovered on the subsequent tube banks.

At the levels D—D and E—E of Figure 1 the tubes of bank 54 are spaced apart and hence the hot gases may pass outwardly between them as at 59. At the portion 58 of tube 54, the spacing increases, but they are sufficiently close together to provide adequate support for the refractory cone 52. Likewise, at the portion 61 of the tubes of bank 54, the tubes spread out and any portion 75 of ore which is carried by the gases and falls be-

tween the tubes at 59 (level D—D) may again fall back between the tubes at 61, near the bottom of the furnace. This is indicated by the arrows 66. At the level E—E the boiler tube portion 59 and the fin 64 serve to retain the main body of ore which collects at the column as shown at 68. The angle of the cone shape formed by portion 61 of tubes 54 is less than the angle of repose of the hot ore within the bottom 70, and hence facilitates passage of the ore between the tubes at the bottom of the furnace.

At the lower end of the tube section 45 of the furnace, there is a converging bottom 70 which serves to close the bottom of the furnace and at the central point of the conical bottom 70 there is provided a treated-ore outlet generally designated 72 consisting of a delivery tube 73 provided with a worm 74 for gradually drawing out of the furnace the finished ore which collects in column 68 over the conical bottom 70.

The hot gases of the furnace result from the flame 75 projecting downwardly from nozzle 50 and the gases travel downwardly through the central opening 76 and thence outwardly between the tubes of bank 54, as indicated by the arrows 77. The combustion of residual gases may be caused to take place just outside tube bank 54, as previously noted. The hot gases then blow over a plurality of additional tubes which may contain either water or air, depending upon process requirements. Thus, for example, in the illustrated embodiment of the invention, there is provided a hot air manifold 80 which is attached to the cylindrical side wall 45 of the furnace and a cold air manifold 81 which is attached to the conical bottom. From the hot air manifold 80 there extend a plurality of air-carrying tubes generally designated 82 which extend inwardly and downwardly into the circular tube bank at 83, thence vertically downwardly and then outwardly and downwardly to the cold air manifold 81. Likewise, attached to the cylindrical side wall 45, there is a water header 85 and a steam header 86 and between these drums there are connected a plurality of banks of tubes, one bank 87 of these tubes being arranged so that the tubes lie alternately in spaced relation with the tube 82 in the bank 83, whereas the remaining banks of steam tubes 88 and 89 are arranged in circles of successively greater diameter. A baffle is arranged as illustrated at 90 for causing the hot gases to flow downwardly as indicated by the arrows 77 so as to traverse the steam and air tubes and thence upwardly as indicated by the arrows 91, 92, 93 and 94 into the stack manifold 95.

The number, spacing and character of tubes in the several banks depend upon the process requirements. Thus, sufficient tube area is provided so as to furnish all hot air needed for the burners, combustion, drying etc. and sufficient steam surface is then provided to recapture the heating values remaining, any surplus steam, above process requirements being used for power.

#### ORE REDUCING SMELTING FURNACE

The furnace apparatus, illustrated in Figures 4 and 5, is essentially the same as that illustrated in Figures 1-3 except that the heat exchanger section 44 of the latter is not used and the reverberating furnace portion 40 is superimposed upon an annular open hearth or annular ring of open hearths. Thus, the furnace section above line G—G of Figure 4 corresponds to the reverberating furnace section 40 of the apparatus shown in Figure 1, and is used for the pre-heat-

ing and reduction of ore to the metallic state, which then falls into the lower open hearth section illustrated in Figure 4 for reducing the metal and gangue to the fluid state so these components may be withdrawn separately.

The furnace illustrated in Figure 4 consists of a base 100 and supporting framework of I-beams 101. At the top of the I-beams there is a roof 102 over a hopper generally designated 105 which may be of any suitable construction, for example of the type illustrated and described with reference to the furnace of Figure 1. An ore introduction pipe 106 is provided in the roof and serves to deposit the ore, generally designated O, into the hopper 105. The hopper 105 delivers the ore through a plurality of spouts 107 to an ore-feeding mechanism of any suitable design, for example such as illustrated and described at 25 in the apparatus of Figure 1. Connected to the columns 101 is an intermediate truss 109 which serves to stiffen the framework and support intermediate columns 110 upon which the furnace proper is built.

The furnace consists of a brick or masonry base generally designated 112 having a built-in circular flue 113 which is connected by breeching 114 to a flue gas exhaust fan or stack (not illustrated). Extending upwardly at the center of the base, there is a masonry pillar 115 having an outwardly diverging under surface 116, an area of maximum diameter 117 and an upper conical dome 118. A water drum 119 may be included centrally within the pillar so as to cool it, and thus keep the pillar from disintegration. An outer wall 120 is built up around the periphery of the base 112 and an intermediate wall 122 extends upwardly to support the roof 123, which is provided with a central opening for the powdered fuel or liquid fuel burner 125. The wall 122 forms the enclosure in which reverberating radiant energy from flame 126 serves to heat the ore and furnace charge particles, as they fall. The height of the wall 122 is accordingly varied in accordance with the temperature conditions sought to be produced on the ore and size of the ore being treated. The roof 123 which may be supported by any suitable structural steel framework (not shown) is provided with openings for receiving the spouts 30 of the ore-feeding mechanism, all as described with reference to Figures 1-3.

Within the outer wall 120 and lying vertically around the periphery of the base, there are a plurality of hearths, four being illustrated in the present apparatus, although a greater or lesser number or a single hearth of any desired shape might be used. Thus, as shown in Figures 4 and 5, there is a hearth generally designated 128, the second identical hearth 129, a third hearth 130 and a fourth hearth 132. Only a portion of hearth 130 and none of hearth 132 show in Figure 5. Each of the hearths has a curved bottom surface 134, Figure 4, extending from the inner wall 135 of the pillar 115, to the outer wall 120. Hearth 129, Figure 5, is representative of all of the hearths.

Hearth 129 is in the form of a segmental basin, having upwardly sloping edge walls 136 and 137, back wall 138 and front wall 139. Similarly, hearth 128 has upwardly sloping walls 140, 141, 142 and another upwardly sloping wall, not illustrated in Figure 5, opposite wall 141. Likewise, Figure 5 illustrates a portion of hearth 130, wherein in the front upwardly sloping wall is designated 144 and the upwardly sloping side wall is designated 145. The side wall 137 of hearth 129 and the side wall 145 of hearth 130 blend into each

other at the elevated land 148 which extends from the inner surface 135 of the pillar 115 to the opposite inner surface 149 of the pier of wall 122. Wall 122 extends downwardly to meet the hearth refractory at that point, as illustrated by the pillars in section in Figure 5.

Between the outer surface 150 of the furnace wall 122 and the inner surface of the outer furnace wall 120 and between side walls 145 and 137 of adjacent hearths 129 and 130, there is an annular space across which there extends a flue opening, generally designated 157, Figure 4. Space 157 joins with vertical flue 151. There is a similar flue opening 152 between the sloping side walls 136 and 141 of hearths 129 and 128 respectively, and a similar elevated land 153 lies between these walls (between the center pillar 115 and the furnace wall 122). Similar flue openings and lands are between each of the remaining hearths (see Figure 5 wherein the flues are designated 154 and 155).

The hearths are covered by the furnace top illustrated at 160, the top preferably being curved over each hearth for strength and also to assist in establishing a condition of reverberating heat energy in the hearth. The flue gases flow through the space 157 and thence downwardly into the flues 151, 152, 154 and 155 as the case may be and thence into circular flue 113, from which they are withdrawn at breeching 114. The gases thence flow into heat exchangers, boilers and the like, not illustrated. Each of the hearths is provided with a tap opening 161 and a spout 162 as illustrated in Figure 4. One or more burner nozzles 164 is provided above the bath of melted ore and slag in each hearth.

#### OPERATION OF ORE TREATING FURNACE

To place the furnace, illustrated in Figures 1-3, into operation, the ore is first introduced into the hopper generally designated 19 by means of inlet pipe 13, and the feed mechanism 25 is placed in readiness for operation. The burner 50 is then lighted and the furnace brought up to temperature.

The furnace may be used for the heat treatment and processing of various ores such as the reduction of finely ground carbonate, sulphide or sulphate ores to the oxides, in a neutral or oxidizing atmosphere and in any required temperature range. The use of the furnace for the reduction of iron ores will be described in detail and may be taken as typical of the operation of the furnace.

##### A. Low temperature reduction of iron ore

For low temperature reduction of iron ores, the furnace flame and height of the furnace are adjusted so that the ore particles are heated to a relatively low temperature in the range of 650° to 800° F. Such temperature suffices for the reduction of weakly magnetic or non-magnetic oxides to the magnetic oxides, preparatory to magnetic concentration of the oxide.

Carbonaceous material, preferably lignitic material, which is finely pulverized is added to the finely pulverized ore as provided for in my Patent No. 2,269,465 and in my co-pending application Serial No. 410,474, now Patent No. 2,333,111 dated November 2, 1943. The carbonaceous material supplies the reducing influence.

The furnace is first brought up to the required temperature by flame 75 which is operated with a minimum air supply to obtain complete combustion, the air being pre-heated by exhaust gases of the furnace so as to provide as high a flame

temperature as possible. In this way there is produced a high radiant energy potential between the flame and the ore processed in the furnace. The ore feeders 25 are then started and the ore mixed with carbonaceous material is dropped in a thin and tenuous "curtain" around the flame 75 through the reverberatory furnace zone 40. The falling material is exposed to the radiant energy of the flame and reverberatory action in the furnace and is brought up to the reaction temperature by the exposure of the particles to the radiant energy. This is accomplished practically instantaneously. In addition, some heat is imparted to the particles by the hot atmosphere of the furnace. The lignitic carbon or non-carbonaceous material is oxidized by the oxide components of the ore, yielding carbon monoxide which in itself acts as a reducing agent as outlined in my patent and my copending application, previously referred to, to reduce or partially reduce the ore and thus make it susceptible to magnetic separation. The ore drops through the conical section, outlet 53 and to the bottom of the furnace in the direction of the arrow 68 where it is slowly withdrawn from the column of ore supported by boiler tubes 59 and the intervening fins 64 between the tubes.

The hot gases pass outwardly between the boiler tubes, above the baffle 64 and thence pass downwardly over the banks of tubes 83, 87, 88 and 89, and thence upwardly between the baffle 90 and the outer refractory line wall 45 of the heat exchanger. The thus cooled gases pass to the flue breeching 95 and may then be carried to further heat exchange apparatus recovering the heat values of the gases, or may be passed over the incoming ore for somewhat pre-heating and drying the ore. The proportion of tube surface in the heat exchanger 44, which is devoted to steam generation and pre-heating of air, may be varied as desired. Thus, one or more of the banks of tubes 87, 88 and 89 may be given over to the heating of air if the process requirements so indicate.

The flow of hot gases through section 59 of boiler tubes 54 carries some finer particles of ore into the space between baffle 90 and the tubes. Such portions of ore tend to fall downwardly rather than to be carried up by the flue gases and the ore particles thus fall upon the lower conical bottom 70 and fall between portions 61 of the tube bank 54 onto the treated ore cone collected in the conical bottom 70. The rotation of screw 74 serves to withdraw the treated ore from the bottom 70, and the speed of withdrawal is adjusted so that a solid column of ore is at all times maintained below level E—E of Figure 1, with the result that the furnace gases are compelled to pass outwardly between the tubes above the fin 64. After withdrawal from the furnace, the ore may be separated by any conventional magnetic or other types of separators for removing the magnetite ore from the accompanying gangue, where the furnace is used for preparing iron ore for magnetic separation. For other uses, the treated ore follows appropriate melting procedures in subsequent steps.

##### B. High temperature reduction of iron ore

A higher grade and more useful concentrate can, however, be obtained by operation at a temperature such that the ore and carbonaceous material fed is heated to a temperature in excess of 1700° F. which is adequate to reduce the oxide to the metallic state, or partially to the metallic

state. The apparatus and operation is the same as that outlined under low temperature reduction except that the heat input of flame 75, the size of particles fed and furnace height are selected so as to allow the particles of furnace charge to be heated to a much higher temperature, viz. in excess of 1700° F., preferably 1800° to 2200° F.

Under such conditions the exit gas temperature at breeching 95 will be correspondingly higher, admitting of a correspondingly higher air preheat to the flame 75 and much higher radiant energy potential between the flame and falling particles of charge fed into the furnace. At this higher temperature there is a reaction between the carbon introduced with the ore and any moisture in the furnace entering with the air, fuel and ore, or that may be introduced as steam. The water vapor reacts with the carbonaceous material present, liberating hydrogen and carbon monoxide in any desired and regulated amounts.

Heating to such a higher temperature, viz. in excess of 1700° F., preferably 1800° F. to 2200° F., causes the finely divided iron oxide particles to be subjected to a hot and highly reducing atmosphere, and the ore particles are reduced to the metallic state almost instantaneously, well within the time needed for such particles to fall the height of the furnace which, of course, is adjusted to the required height for any given size ore being processed. For many purposes of the invention, it is not necessary that the particles be completely reduced to the metallic state. Thus it is sufficient for magnetic separation and other uses to only partially metallize the oxide, thus in effect forming a metallic shell with an oxide core. Such partially metallized material can then be concentrated magnetically or by other methods of concentration. Such concentrates may also have an increased iron concentration, the iron content being adjusted to any concentration desired. Such concentrates may be used for blast furnace charges and can also be used directly or indirectly in the open hearth furnace or a modification of same, thus by-passing the blast furnace.

The increased heat in the exit gases can be completely utilized. Some of the available heat is required for the preheating of combustion air used in the apparatus and the remaining heat may be used to generate power for the grinding of the ore and fuel and other power purposes and the pre-drying of the ore, if required. It is contemplated that the heating value of any combustibles in the flue gases shall be recovered by adding superheated air to oxidize the residual combustibles in an enlargement of the space between tube bank 54 (at 59) and the tube row 83, where the gases are still above the temperature of ignition.

Among the advantages of high temperature treatment of the iron ore is the increased value of the product, the generation of hydrogen as well as CO as reducing gases, vastly increased reaction rate (due to the presence of the hydrogen and the increased temperature), and the production of a product which is much more readily separated from the gangue.

While the high temperature process is least usable for ores having very low softening-point gangue material, the gangue in most ores, for example siliceous ores, will not be seriously affected or soften at the temperature indicated.

The method of heating by radiant energy provides in addition a differential rate of heating of ore and gangue, the ore heating faster than the 75 by means of inlet pipe 106, and after the hopper

gangue material because of the difference in absorptive values of the surfaces of such diverse materials. This causes the gangue to drop to the relatively cooler section of the furnace before attaining a temperature that will produce softening and consequent agglomeration.

It will be noted that the top of the reaction chamber will be substantially hotter due to stratification with the hotter and lighter gases at the top, and due to the radiant energy reverberating effects which are obtained in this zone. For a similar reason the lighter hydrogen and CO will tend to remain in the reaction chamber while the heavier inert gases flow out at the bottom. This is a major advantage of the invention.

#### OPERATION OF REDUCING SMELTING FURNACE

In operating the apparatus of Figures 4 and 5 for the reduction of iron ore, the process and reactions are as described with reference to Figures 1-3 except that higher temperatures and higher concentrations of reducing gases may be used to obtain complete reduction of the oxides. It will be noted that in reduction of iron ore by the combined process carried out in the apparatus of Figures 4 and 5, the full utilization of the heat values in the fuel is provided for, including the recovery of the heat values in the residual combustible gases from the reducing section 122 of the furnace. By utilizing high temperatures, viz. from 1800° to 2200° F. for the charge, and an adequate amount of carbonaceous material as described in my Patent No. 2,269,465 and my co-pending application Serial No. 410,474 or other carbonaceous material, the ore particles falling through chamber 122 are completely reduced prior to their entry into the open hearth section at the bottom of the furnace.

Due to the higher temperatures of operation and the heat input by way of the hearth burners 164, the gases at flue 114 contain a large amount of heat, which may be recovered for the heating of the combustion air and generation of steam and power. This is accomplished in an independent heat exchanger section not indicated.

With most ores, flux is required to obtain sufficient fluidity of the slag. The flux may be mixed with the ore, preferably as a finely divided powdered oxide of lime, which is dropped through the furnace along with the ore and carbonaceous material.

While the furnace apparatus of Figures 4 and 5 may be employed in direct reduction of higher grade iron ores and concentrated ores, it is also adapted for the utilization of low grade ores, particularly making possible smelting and utilization of iron ores with 30% or less of iron content without concentration. The furnace is thus adaptable for installation adjacent low grade ore deposits, the only freight charges involved being against the fuel, flux and metallic product, minor items in most cases. The furnace thus makes possible the working of smaller deposits and wider distribution of steel-making, and the products of the furnace are available for small open hearth and furnace installations, variously located.

In placing the furnace in operation, the burner 125 and the several burners 164 over the hearths 70 are lighted and the furnace brought up to temperature. At the same time water circulation through the drum 119 is started so as to maintain the interior of the column 115 relatively cool. The ore is then introduced into the hopper 105 by means of inlet pipe 106, and after the hopper

has been filled sufficiently, the ore-feeding mechanism 25 is started, whereupon the ore, together with any flux material falls as a "curtain" around the intensely hot, brilliant flame 126 projected downwardly from the burner 125. As the ore and flux falls, it absorbs radiant energy from the flame and is heated almost instantaneously. In this connection, it should be borne in mind that conduction is not required for the transmission of heat energy from the flame 126 to the curtain of falling particles of ore and flux. Conduction of heat to the particles does play some part in heating the ore particles, but by far the greatest heating effect is due to absorption of the radiant reverberating energy on the particles of ore and other components of the charge. The ore particles fall into the space 165 between the outer surface of the pillar 115 and between the inner surface of the wall 122 and any ore particles which fall upon the slope of cone 118 likewise slide or, if fluid, drip downwardly into this space and into the hearths below. The gases produced by flame 126 likewise pass downwardly through space 165 and into the hearths, where any residual combustible is oxidized, imparting additional heat to the material. Additional heat is supplied by the flame or series of flames from burners 164, combustion conditions being adjusted to a relatively neutral (slightly reducing or slightly oxidizing) atmosphere, in accordance with the requirements of the metal and slag bath and the amount of oxygen required to oxidize the combustibles in the gases from the reducing furnace section 122 above the hearths. Within the hearths the ore particles are melted, if not already melted due to the radiant heat energy absorbed in section 122, and the ore is then rendered fluid and the ore smelted by the reverberating heated gases above the ore. The resultant metal collects at 166 in the bottom of the hearth. Periodically the ore and slag are drawn off through the tap holes 161 of each of the hearths, and after each tapping the tap hole is plugged in the conventional manner. Separate tap holes for ore and slag may be provided.

The spent gases from the hearths are drawn out through ports 157 on each side of each hearth down into duct 113 and through heat exchangers, not indicated, where part of the heat is utilized for pre-heating the air for the various burners and for making steam for furnishing power to grind the ore and fuel, and other purposes including pre-drying the ore if required, thus effectively utilizing all the heat.

With this process, ore having an iron content of 30% can be reduced to a metallic iron with less total fuel per ton of metal than is required in standard blast furnace practice for the blast furnace alone, operating on high grade ores, and permits a much higher heat recovery, more than ample for all power purposes including the grinding of ore and fuel. In addition, the total fuel for the burners as well as for the carbonaceous reducing agent mixed with the ore, can be any low sulphur coal and/or lignite. The metal produced is available for electric furnace and open hearth use and refining.

It provides a means for the economical utilization of low grade ores and scattered deposits of same on a competitive basis with high grade ores.

By "finely divided" ore, as used herein, there is meant a fineness of particle size sufficient, on the average, completely to free the particles of oxide from associated particles of gangue, so that concentration may be accomplished by customary

processes such as magnetic separation, flotation or the like. For example, a fineness of 100 mesh or finer is suitable for most ores, although larger sizes are frequently permissible for utilization in the processes herein. The invention is not limited to any particular degree of fineness, for the criteria is the time element required for heating the ore particles by reverberatory radiant heat energy while the particles are falling through a given height of furnace. The furnace height is therefore selected, in any particular installation, so as to allow sufficient time of fall for heating particles of the size being processed.

Ores of the required fineness may be those occurring naturally or there may be used the ore dumps from previous concentration processes or ore ground and graded to the selected sizes suitable for a particular furnace.

As many apparently different embodiments of this invention may be made without departing from the spirit and scope thereof, it is to be understood that I do not limit myself to the specific embodiments herein except as defined by the appended claims.

What I claim is:

1. In an ore treating process wherein ore is heated to an elevated temperature, the improvement which comprises projecting a luminescent flame downwardly along a vertical axis of an enclosed vertical space and substantially continuously dropping ore particles downwardly in a manner so as to form a curtain of falling particles around said flame for absorbing heat radiated therefrom and simultaneously projecting flame jets transversely through said curtain of falling particles to consolidate them.

2. The process of smelting iron ore "fines" which comprises projecting a flame along the vertical axis of an enclosed vertical furnace to produce a condition of reverberating radiant heat energy in said space, substantially continuously dropping a furnace charge mixture of iron ore "fines," finely divided solid reducing agent and finely divided flux downwardly in said space around said flame in a manner so as to form a curtain of falling particles of the furnace charge around the flame and in direct view thereof for absorbing heat radiated therefrom, collecting the so treated and heated furnace charge mixture in a lower refining furnace hearth and therein further heating the charge to render the iron and resultant slag fluid.

3. An ore reducing furnace comprising a vertical space connected at its lower end to a lower reverberating furnace located beneath said vertical space, a burner for projecting a flame downwardly along a central axis of said vertical space, means for feeding a finely divided furnace charge into the upper part of said space in a position to allow said charge to fall vertically around said flame, and additional burner means for heating said lower reverberating furnace.

4. An ore reducing furnace comprising a relatively tall cylindrical space enclosed at its upper end and having an annular bottom opening at its lower end leading into a reverberating furnace space located directly beneath said cylindrical space, burner means mounted on the upper end of said cylindrical space and positioned for projecting a flame downwardly along a central vertical axis thereof, means positioned on the upper end of said cylindrical space for substantially continuously dropping finely divided ore particles of ore charge into the cylindrical space substantially over said annular opening, means in the

reverberating furnace space for supplying heat thereto and for withdrawing the so treated ore charge at a rate sufficient to prevent any substantial accumulation of ore charge in the cylindrical space.

5. An apparatus of the type described in claim 4 wherein the reverberating furnace space is annular.

6. An apparatus of the type described in claim 4 wherein the reverberating furnace space is composed of a plurality of segmental arcuate hearths having outlet flue openings therebetween.

7. An ore reducing furnace comprising a closed-top vertical space forming a reaction zone, a burner for projecting a flame downwardly along a central axis of said zone, ore-feeding means at the top of said zone for dropping fine ore particles downwardly around the central axis in a manner so as to form a curtain of falling ore particles around the flame along said axis, and a plurality of radial segmental hearths beneath said reaction zone, each being provided with a heat burner, draw-off port and exhaust flue, said hearths being positioned to catch the reacted ore particles after they have fallen in a curtain through said reaction zone.

8. The method of reducing iron ore comprising establishing a central flame source of high radiant energy potential in a reverberatory space, selecting a finely divided ore, mixing said ore with finely divided carbonaceous material to form a furnace charge, dropping said charge as a curtain of particles around said flame source of high radiant energy potential and subjecting said curtain of particles directly to said radiant energy potential so as to heat the charge to reaction temperature principally by means of radiant energy while said charge remains dispersed, said temperature being sufficient for the reduction reaction by radiant and reverberatory heat energy while the furnace charge falls by gravity freely dispersed in the atmosphere of said heated reverberatory furnace space.

9. The method of preparing finely divided iron ore for subsequent concentration comprising establishing a central flame source of high radiant energy potential in the reverberatory space, mixing said ore with a minor percentage of finely divided carbonaceous matter to form a furnace charge, dropping said charge as a curtain of particles around said flame source of high radiant energy potential and subjecting said charge to direct radiant energy from said flame source of high radiant energy potential so as to heat said charge principally by radiant energy to a reaction temperature in excess of 1700° F. for the reduction reaction by radiant and reverberatory heat energy while the charge falls by gravity freely dispersed in a reducing atmosphere in said heated reverberatory furnace space at least partially to metallize the ore.

10. The method of utilizing low-grade, finely-divided ore which comprises establishing a central flame source of high radiant energy potential in a reverberatory space, mixing said ore with finely-divided carbonaceous material to form a furnace charge, dropping said charge as a curtain of particles around said flame source of high radiant energy potential, subjecting said curtain of particles to direct radiant energy from said flame source of high radiant energy potential so as to heat said charge principally by radiant energy to a temperature sufficient to allow reduction

of the ore while the particles of furnace charge fall freely by gravity dispersed from each other in a reducing atmosphere in a heat reverberatory furnace space, collecting the heated and reduced ore in a reverberatory heated hearth below said furnace space to complete the reduction and smelting of the ore of the furnace charge.

5. In an ore treating process wherein ore is heated to an elevated temperature, the improvement which comprises projecting a luminescent flame downwardly along a vertical axis of an enclosed space to maintain a high temperature zone in the uppermost portion of said space and progressively cooler zones in the lower portion of said space, introducing a mixture of ore particles and a finely divided solid reducing agent substantially continuously into said high temperature zone at the top of said enclosed space, thereby maintaining a body of reducing gases in said high temperature zone and dropping said ore particles downwardly in a manner so as to form a curtain of falling particles around said flame and in direct view thereof for absorbing heat radiated therefrom whereby said ore particles are heated to an elevated temperature and reduced in said high temperature zone.

10. In an ore treating process wherein ore is heated to an elevated temperature, the improvement which comprises projecting a luminescent flame downwardly along a vertical axis of an enclosed space to maintain a high temperature zone in the uppermost portion of said space and progressively cooler zones in the lower portion of said space, introducing a mixture of ore particles and a finely divided solid reducing agent substantially continuously into said high temperature zone at the top of said enclosed space, thereby maintaining a body of reducing gases in said high temperature zone, dropping said ore particles downwardly in a manner so as to form a curtain of falling particles around said flame and in direct view thereof for absorbing heat radiated therefrom to heat said ore particles to an elevated temperature in said high temperature zone and reduce said particles, collecting the heated and reduced ore below said enclosed space, and smelting said heated and reduced ore.

HENRY G. LYKKEN.

#### REFERENCES CITED

The following references are of record in the file of this patent:

#### UNITED STATES PATENTS

| Number    | Name            | Date           |
|-----------|-----------------|----------------|
| 244,408   | Weimer          | July 19, 1881  |
| 285,462   | Canavan         | Sept. 25, 1883 |
| 555,680   | Cunningham      | Mar. 3, 1896   |
| 806,774   | Brown           | Dec. 12, 1904  |
| 817,414   | Brown           | Apr. 10, 1906  |
| 1,278,180 | McDonald        | Sept. 10, 1918 |
| 1,283,515 | Hill            | Nov. 5, 1918   |
| 1,618,011 | Isenberg et al. | Feb. 15, 1927  |
| 2,052,928 | Harris          | Sept. 1, 1936  |
| 2,194,454 | Greenwalt       | Mar. 19, 1940  |
| 2,365,194 | Hodson          | Dec. 14, 1944  |
| 2,418,394 | Brown           | Apr. 1, 1947   |

#### FOREIGN PATENTS

| Number  | Country       | Date                            |
|---------|---------------|---------------------------------|
| 663,942 | France        | Aug. 27, 1929                   |
| 268,793 | Great Britain | Mar. 31, 1927<br>(Not accepted) |

Patent No. 2,503,555

**Certificate of Correction**

**HENRY G. LYKKEN**

April 11, 1950

It is hereby certified that errors appear in the printed specification of the above numbered patent requiring correction as follows:

Column 2, line 36, for "plates 15 and 16" read *plates 15 and 18*; column 6, line 53, for the word "hearts" read *hearths*;

and that the said Letters Patent should be read with these corrections therein that the same may conform to the record of the case in the Patent Office.

Signed and sealed this 18th day of July, A. D. 1950.

[SEAL]

**JOE E. DANIELS,**  
*Assistant Commissioner of Patents.*